

# UNITED STATES PATENT OFFICE.

JAMES HEBER PARKER, OF READING, AND BERTON H. DE LONG, OF SPRINGMONT, PENNSYLVANIA, ASSIGNEES TO CARPENTER STEEL COMPANY, OF READING, PENNSYLVANIA, A CORPORATION OF PENNSYLVANIA.

## ALLOY TOOL-STEEL.

1,233,118.

Specification of Letters Patent. Patented July 10, 1917.

No Drawing.

Application filed June 26, 1916. Serial No. 105,855.

*To all whom it may concern:*

Be it known that we, JAMES HEBER PARKER and BERTON H. DE LONG, both citizens of the United States, residing at, respectively, Reading and Springmont, in the county of Berks and State of Pennsylvania, have invented certain new and useful Improvements in Alloy Tool-Steels, of which the following is a specification.

10 Our invention relates to high speed alloy tool-steels; and our purpose is to provide an improved alloy steel of this class adapted to extend the limits of possible speed and cut, and to secure maximum service within 15 these limits, while at the same time providing such malleability and machining qualities as will permit of satisfactory shaping for various uses.

Our invention contemplates the production 20 of an alloy high speed tool steel of the tungsten-chromium-vanadium type, having as a novel feature a distinctively high proportion of cobalt which makes possible the securing of desired characteristic qualities 25 in such degree as have not heretofore been attained,—to wit: malleability; machining softness; and, when treated, red-hardness, with maximum serviceability.

As actually employed by us with very 30 satisfactory results, our improved alloy steel contains the following elements in about percentages as stated, to wit:

|          |         |
|----------|---------|
| Carbon   | 0.35%   |
| Vanadium | 2.00%   |
| Chromium | 3.50%   |
| Tungsten | 12.00%  |
| Cobalt   | 30.00%  |
| Iron     | 52.15%  |
|          | 100.00% |

It will be seen that this alloy forms a tungsten steel, having ordinary percentages of tungsten and the quantitatively minor

elements, but characterized by the use of 45 cobalt with iron in quantities forming jointly the great bulk of the alloy and proportioned approximately one part of cobalt to two parts of iron.

These proportions of iron and cobalt correspond substantially with the eutectic proportions which provide the lowest fusing point for the compound relative to the fusing points of its component elements. These main elements may be advantageously 55 employed with such variations in the other elements and their proportions as have heretofore been used, with effects similar in character to those secured by such variations as ordinarily employed. The characteristic features of our improved high speed alloy tool-steel is the use of iron and cobalt in substantially eutectic proportions as stated and constituting the great bulk of the alloy; the distinguishing effect being the securing 65 of maximum service, with increase of possible speed and cut, and in connection with capability for requisite shaping operations.

What we claim is:

1. A tungsten-steel having a base composed of between 30% and 45% of cobalt and between 55% and 70% of iron, said compound constituting the bulk of the alloy and the tungsten between 8% and 20% thereof. 70

2. An alloy tool-steel composed mainly of iron and cobalt proportioned approximately two of iron to one of cobalt, 8% to 20% of tungsten and .5% to 2.5% of vanadium. 75

3. An alloy tool-steel composed mainly of 80 iron and cobalt proportioned approximately two of iron to one of cobalt, 8% to 20% of tungsten and .5% to 2.5% of vanadium and 1% to 6% of chromium.

In testimony whereof we affix our signatures.

JAMES HEBER PARKER.  
BERTON H. DE LONG.